

Patented Sept. 2, 1952

2,609,308

# UNITED STATES PATENT OFFICE

2,609,308

## METHOD AND MATERIAL FOR PRODUCING COATINGS ON METAL

Robert C. Gibson, Birmingham, Mich., assignor to Parker Rust Proof Company, Detroit, Mich.

No Drawing. Application November 22, 1947,  
Serial No. 787,621

9 Claims. (Cl. 148—6.17)

1

This invention relates to a method and material for producing phosphate coatings on metals.

More particularly it relates to a method of producing predominately iron phosphate coatings possessing a combination of properties heretofore unknown.

Methods for obtaining ferrous phosphate coatings on metals have been known for many years. This is illustrated by United States Patent No. 870,839 issued November 12th, 1907 to Coslett. He used a boiling solution of phosphoric acid with some iron dissolved therein and into which the articles were immersed and left until the coating formed. The processing was continued until the coating action ceased, as shown by cessation of bubbling, usually requiring over an hour. The completed coating weighed upwards of 1000 milligrams per square foot of surface treated.

Later developments added refinements to Coslett's method. It was found that the presence of other metals such as manganese added to the bath increased the corrosion resistance somewhat. Copper in small amounts was found to speed up the coating action, and the presence of certain oxidizing agents was found not only to reduce the time for producing a substantially continuous coating, but also that stage was reached while the coating was much thinner. This is illustrated in United States Patent 1,911,726 issued May 30, 1933, to Tanner and Lodeesen. The coatings produced commercially under that patent that averaged to have not more than one-sixth the thickness of the average coating produced under the Coslett patent.

In all of these developments, solutions of dihydrogen phosphates of metals whose less acid phosphates are insoluble in water have been required. There are certain properties common to all of these coating chemicals. The dihydrogen phosphates of these metals are decidedly acid, usually developing a pH value of lower than 3 in the coating solution, depending upon the strength of solution and the temperature. They all produce coatings better and more rapidly when the solution is fresh, but the solution hydrolyzes on being heated, and in so doing produces less acid phosphates which are thrown down as a sludge, leaving the solution more acid than when the dihydrogen phosphate is first dissolved. Agitation, such as obtained by spraying, accelerates hydrolysis with the inevitable production of free phosphoric acid in the solution. This acid cannot be neutralized without the formation of additional sludge by further hydrolysis, and release of more free acid.

When metal is first cleaned with strongly acid or alkaline solutions the phosphate coating tends to be deposited in the form of large crystals which render the coating unuseable for certain applications. This condition can be avoided only by adding extra steps to the procedure.

2

It is customary with all commercial phosphate solutions to heat them in order to obtain a satisfactory reaction with the metal. This is usually done with steam coils immersed in the solution. The sludge mentioned above gradually forms a crust on the coils so that heat transfer is retarded and the coils must be removed and cleaned at frequent intervals. The sludge also causes difficulties, especially in installations where the solution is sprayed and recirculated, by plugging nozzles and pipes, thus necessitating additional maintenance cost.

An object of this invention is the production of an iron phosphate coating without forming more than a negligible amount of sludge.

Another object is the formation in a short time of an extremely thin coating which is equivalent to the usual thicker phosphate coatings as a paint base.

20 A further object is to provide a method of treatment whereby the pH of the solution automatically remains high, thus avoiding the necessity for continued adjustment.

Other objects will become apparent as the description proceeds.

It is known that the dihydrogen phosphates of the alkali metals, including ammonium, do not possess any direct coating ability because their less acid phosphates are all water soluble. Where alkali metals are mentioned hereinafter the term includes ammonium. They do however produce a small amount of free phosphoric acid in aqueous solution and this will attack a metal surface and produce a small amount of coating which has been shown by many tests to add only slightly to the paint retaining ability of the surface.

These particular phosphates nevertheless have certain highly desirable characteristics which are made use of in combination with my invention. They of themselves form no sludge. They also have a pH in solution which is substantially higher than that developed by the acid phosphates of zinc, iron and manganese for example. This is important both from the standpoint of economy of operation and in avoiding certain production difficulties. There is much less metal dissolved during treatment and the formation of rust on the coated metal from steam during line stoppage is substantially eliminated. This has always been a source of trouble with solutions which operate in a low pH range.

40 The low acidity is apparently very effective in precipitating the dissolved iron immediately as coating since practically no dissolved iron is found in the solution. Furthermore the original pH of the bath actually rises somewhat in the initial stages of use rather than becoming lower, as in solutions of phosphates of coating metals, and as would be expected in this case as iron accumulates.

45 The process of my invention may be used in combination with unusually alkaline or acid cleaning solutions. The normal tendency under

such conditions is for the coating to exhibit "sparkle," which is caused by unusually coarse crystals. This is minimized by the present invention since the resulting coatings are fine grained.

The invention resides in the discovery that if an oxidizing agent is added to solution of dihydrogen phosphate of an alkali metal, a coating of increased thickness is formed, exactly the opposite of the effect of similar agents with phosphates of coating metals, and some alteration in the physical or chemical structure of the coating occurs which greatly augments its value as a paint base to the point where it is equal to the much heavier coating obtained with the standard phosphate process customarily used. Moreover these results are accomplished with a coating weight which is unusually low. This is highly important in maintaining maximum paint luster and also where it is desired to paint a coated sheet and thereafter form it to the desired shape. Heavier coatings, for example weighing over 100 milligrams per square foot of surface treated, are totally unsuitable for some such forming operations. Initial adhesion of certain types of paint has been found to be superior to that obtained with heavier coatings.

Investigation has shown that there are certain limitations that must be observed if maximum benefit of the invention is to be obtained. The pH of the operating solution should not be substantially lower than that normally obtained by the dihydrogen phosphate of the alkali metal, or 4.2. Increased acidity over that amount given gives inferior results in paint adhesion. The total concentration of the bath both in respect to the phosphate and oxidizing agent have a bearing on ultimate results obtained. Different oxidizing agents are effective in different amounts, but in each case a minimum is required to cause the necessary change in coating structure in order to obtain best results. For example if chlorate is used there appears a rather sharp improvement in results when .5%  $\text{ClO}_3$  is present. The amount of the oxidizing radical is given herein whenever not otherwise specified, since it is of the amount of this radical which is essential regardless of the atomic weight of the base united therewith. Higher amounts may be used up to at least 4%, and sometimes even more, with some added improvement but at least .5% should be used.

Nitrite is more effective than chlorate in that only a tenth as much is required for equivalent results. Bromate may be used with good results with concentrations ranging from .2 to 2.0%  $\text{BrO}_3$ . Sulfite is likewise effective. A good working range is from .2% to .5%  $\text{SO}_3$ . Apparently the oxidizing agent should be of a kind and quantity that will have about the same effect on the coating action as .5% to 4% of chlorate will have.

Nitrate, one of the most common oxidizing agents used in phosphate coating operations with phosphates of coating chemicals, is substantially without effect in the present instance, probably due to the high pH. Permanganate also is ineffective.

It appears to be characteristic of suitable oxidizing agents in right amounts that they cause an increase in coating weight over that obtained with identical conditions except for their presence. Unsuitable agents or improper amounts of suitable agents do not produce this result.

In spite of this distinction it does not necessarily follow that there is a direct relationship between the amount of coating and the excellence

of paint adhesion. Comparable results, as indicated by salt spray tests, have been obtained with coatings ranging from 65 down to 22 milligrams per square foot of surface treated. The latter value is comparable to that obtained in the absence of any oxidizing agent under some conditions. The quality of the coating produced by this invention is, however, quite distinctive.

A change in the amount of phosphate dissolved in solution likewise causes a change in the pH. There is a concentration of the salt which, for best results, should not be exceeded unless the bath is neutralized to compensate for the increased acidity. I have found that a pH value not lower than approximately 4.2, as obtained with a concentration of sodium dihydrogen phosphate of 14 grams per liter and .5%  $\text{ClO}_3$ , should prevail. Greater amounts of phosphate than this can be used but there appears to be no advantage in a higher concentration, and consumption is increased because of an increased amount of chemicals carried out on the work. Usually the pH value will be substantially higher than 4.2 as a result of reaction with the metal and the presence of salts in ordinary water which react with the phosphate reduce the acidity somewhat.

In a commercial installation a solution was prepared by dissolving in about 900 gallons of water 113 pounds sodium dihydrogen phosphate and sufficient sodium chlorate to furnish .5%  $\text{ClO}_3$ . The solution was heated to 160° F., and emulsion cleaned steel parts were coated therein by spraying for a period of one minute, water rinsed then finally rinsed in a dilute hot mixture of phosphoric and chromic acid. After production had continued for a short time the pH of the solution was found to have reached a value as high as 5.2.

Numerous line stoppages where the coated metal was subjected to hot vapors for extended periods caused no objectionable amount of rusting in any case and in most cases evidence of attack was entirely absent although the coating weight seldom exceeded 60 milligrams per square foot of surface treated.

The sludge which accumulated amounted to only about one-tenth pound for each thousand square feet of surface treated. Ten times that amount may be produced with conventional phosphate treatments. At no time was it necessary to clean the heating coils or spray nozzles.

Chemical consumption amounted to 1.90 lbs. per thousand square feet or about one-half that ordinarily obtained where the majority of the coating is derived from chemicals furnished by dissolved phosphates of zinc, manganese, etc.

The acidified final rinse aids in providing the maximum results in paint adhesion, especially where the oxidizing agent is near its lower effective limit, and forestalls possible difficulties from blistering, which may be caused by the retention of unconverted hard water salts on the coated surface. Where as much as 4% chlorate was included in the solution, the final rinse in phosphoric and chromic acid made little difference in paint adhesion.

A dilute solution of chromic acid or dichromates other than those of the alkali metals may be used instead of the mixture of phosphoric and chromic acids.

Grease emulsifying agents usually employed in metal cleaners may be employed herein. In the particular example given above a mixture of polyoxyethylene sorbitan monooleate and sorbitan monooleate were employed.

A material for preparing and replenishing the solution may be made by mixing the correct proportions of phosphate and oxidizing agent. This may be furnished as a dry combination or as a concentrated aqueous solution. A suitable ratio of phosphate and sodium chlorate to maintain the phosphate substantially constant and the chlorate at approximately .5% is :

|                                           | Pounds |
|-------------------------------------------|--------|
| Sodium dihydrogen phosphate or equivalent | 1.36   |
| Sodium chlorate                           | .53    |

Other compatible phosphates of alkali metals and oxidizing agents may be mixed. Ammonium phosphate and sodium chlorate would form an explosive mixture and so are incompatible for a dry mix, although they may be used together in solution.

To recapitulate, my invention makes use of the dihydrogen phosphates of the alkali metals at pH values not lower than approximately 4.2 and not higher than 6.

Certain oxidizing agents, equivalent to .5% to 4% chlorate, added to the solution have been found to cause an unforeseeable alteration in the coatings over that obtained by the phosphate alone which makes them exceptionally valuable as a paint base. Among these agents are chlorate, nitrite, bromate, and sulfite. These are all characterized by their ability to increase the coating weight over that obtained by the phosphate alone, as well as modifying the quality of the coating, whereas oxidizing agents not suitable, such as nitrate and permanganate, do not exhibit this ability.

Specific examples of solutions have been given to illustrate the invention, it being understood that variations may be made as indicated without departing from the scope of the invention.

The phosphates of different alkali metals may be used, and the base of the chlorate or other oxidizing radical is immaterial provided that it is not of a kind that will interfere with the coating action. No danger of this is present when only alkali metals are present in the oxidizing agent.

In the claims, as well as in the foregoing specification, "alkali metal" is used in its broad sense which includes ammonium.

What I claim is:

1. The process of producing a phosphate coating on a ferrous surface, which consists in applying to the surface a solution consisting essentially of water, acid phosphate of an alkali metal and an oxidizing agent of the group consisting of nitrites, sulphites, chlorates and bromates of the alkali metals, the oxidizing agent being present in an amount having an effect on the quality and rate of coating on the said ferrous surface substantially equal to that produced by .5% to 4% chlorate, and the solution having a pH of from 4.2 to 6, and continuing the application until a coating results.

2. The process of producing a phosphate coating on a ferrous surface, which consists in applying to the surface a solution consisting essentially of water, acid phosphate of an alkali metal and a chlorate of an alkali metal, the chlorate being present in an amount from about .5% to about 4% and the solution having a pH of from 4.2 to 6, and continuing the application until a coating results.

3. The process of treating a ferrous surface to receive a siccative coat which consists in applying to the surface a solution consisting essentially of water, acid phosphate of an alkali metal and

an oxidizing agent selected from the group consisting of nitrites, sulfites, chlorates and bromates of the alkali metals, said oxidizing agent being present in an amount having an effect on the quality and the rate of coating on the said ferrous surface substantially equal to that produced by about .5% to about 4% chlorate ion, said solution having a pH from 4.2 to 6.0; continuing the application until a coating results and thereafter rinsing the said coating in a dilute solution of chromic acid.

4. A process of treating a ferrous surface to receive a siccative coat which consists in applying to the surface a solution consisting essentially of water, acid phosphate of an alkali metal and a chlorate in an amount from about .5% to about 4%, said solution having a pH from 4.2 to 6.0, continuing the application until a coating results and thereafter rinsing the said coating in a dilute solution of chromic acid.

5. A solution for producing a phosphate coating on a ferrous surface which consists essentially of water, acid phosphate of an alkali metal and an oxidizing agent selected from the group consisting of chlorates, bromates, nitrites and sulfites, said chlorate, when present, being present in an amount from .5% to about 4%; said bromate, when present, being present in an amount from .2% to 2.0%; said nitrite, when present, being present in an amount from .05% to about .4%; said sulfite, when present, being present in an amount from .2 to 5%, said solution having a pH from 4.2 to 6.0.

6. A solution for producing a phosphate coating on a ferrous surface which consists essentially of water, acid phosphate of an alkali metal and a chlorate of an alkali metal in an amount from about .5% to about 4%, said solution having a pH from 4.2 to 6.0.

7. A solution for producing a phosphate coating on a ferrous surface which consists essentially of water, acid phosphate of an alkali metal and a nitrite of an alkali metal in an amount from about .05% to about .4%, said solution having a pH from 4.2 to 6.0.

8. A solution for producing a phosphate coating on a ferrous surface which consists essentially of water, acid phosphate of an alkali metal and a sulfite of an alkali metal in an amount from .2% to .5%, said solution having a pH from 4.2 to 6.0.

9. A solution for producing a phosphate coating on a ferrous surface which consists essentially of water, acid phosphate of an alkali metal and a bromate of an alkali metal in an amount from about .2% to 2.0%, said solution having a pH from 4.2 to 6.0.

ROBERT C. GIBSON.

#### REFERENCES CITED

The following references are of record in the file of this patent:

#### UNITED STATES PATENTS

| 65 | Number    | Name            | Date          |
|----|-----------|-----------------|---------------|
|    | 1,320,734 | Chadwick et al. | Nov. 4, 1919  |
|    | 2,132,883 | Romig           | Oct. 11, 1938 |
|    | 2,268,323 | Martin et al.   | Dec. 30, 1941 |
|    | 2,302,510 | Tanner et al.   | Nov. 17, 1942 |
|    | 2,302,643 | Thompson        | Nov. 17, 1942 |
|    | 2,304,299 | Boyle et al.    | Dec. 8, 1942  |
|    | 2,312,855 | Thompson        | Mar. 2, 1943  |
|    | 2,403,426 | Douty et al.    | July 2, 1946  |
|    | 2,477,841 | Ward            | Aug. 2, 1949  |
| 75 | 2,479,423 | Snyder          | Aug. 16, 1949 |